

# United States Patent

[11] 3,617,206

[72] Inventor **Xavier Kowalski**  
Creve Coeur, Mo.  
[21] Appl. No. **854,358**  
[22] Filed **Aug. 27, 1969**  
[45] Patented **Nov. 2, 1971**  
[73] Assignee **Monsanto Company**  
St. Louis, Mo.

[56] **References Cited**  
UNITED STATES PATENTS  
2,735,742 2/1956 Godehn..... 8/137.5  
3,234,124 2/1966 Irani..... 8/137 X  
3,476,505 11/1969 Kirner et al..... 8/139  
3,497,313 2/1970 Quimby..... 8/139

*Primary Examiner*—Mayer Weinblatt  
*Attorneys*—Herbert B. Roberts, James J. Mullen and Neal E. Willis

[54] **PROCESSES FOR SCOURING TEXTILES**  
3 Claims, No Drawings

[52] U.S. Cl..... **8/137,**  
8/137.5, 8/139  
[51] Int. Cl..... **B08b 3/00,**  
D06f  
[50] **Field of Search**..... **8/137,**  
137.5, 139

**ABSTRACT:** Textile fibers which have been desized and are about to be bleached are scoured with a boiling alkaline caustic solution containing a surfactant and a solubilizing agent such as amino tri(methylene phosphonic acid). This process provides fibers with a substantially reduced impurity level and an end product which is substantially more conducive to a subsequent dyeing process.

## PROCESSES FOR SCOURING TEXTILES

## PROCESSES FOR SCOURING TEXTILES

The present invention relates to an improved process for bleaching and dyeing textile materials. Specifically, this invention is concerned with scouring materials with a composition containing an organic material which functions as a solubilizing agent.

Preparing textile materials for dyeing and finishing generally involves a series of well-known steps. The material is first singed to burn off excess fibers, desired to remove any artificial coating put on the material for processing, rinsed, and then it is scoured. After scouring, the material is again rinsed and then, in succession, it is bleached, scoured, rinsed, mercerized, rinsed, dyed or printed, and finished. These steps are more specifically described in *Chemistry and Chemical Technology of Cotton*, Interscience Publishers, Inc., New York, N. Y. 1955, edited by Kyle Ward, Jr., and which is incorporated herein by reference. A discussion per se of the scouring step starts on Page 144 of said publication.

In general, scouring is the fourth major step in the above-described textile finishing process. The purpose of the scouring step is to remove foreign matter left on the textile material after desizing. The foreign matter can be naturally occurring colorants, waxes, and protein, as on a cotton fiber. The foreign matter can also be materials applied to fibers and yarns to improve their manufacture into fabrics, as in weaving or knitting, but which have to be removed prior to dyeing and finishing to insure that the color of the material will be uniform throughout. These materials can be sizes such as starch, polyvinyl alcohol, ethylene maleic anhydride, carboxy methyl cellulose and others, or lubricants such as emulsified oils, softeners, antistatic materials, and others.

The scouring process is desirable in order to attempt to remove impurities or foreign matter and thus ultimately prepare a "whiteness in color" product suitable for subsequent dyeing and effecting a uniformity of color thereon. Generally, commercial scouring or boiling processes involve contacting the textile material with alkaline aqueous solution containing a caustic material such as sodium hydroxide and a surfactant. In the past, however, this type of scouring step was not substantially completely effective in that the subsequently bleached textile material did not exhibit a better than fair whiteness in color. By the practice of the present invention, however, the whiteness of the bleached material is substantially improved.

Accordingly, it is an object of this invention to improve the process of the type described so as to enhance the appearance of the textile material treated and to clean the surface of said material to promote a more effective dyeing step.

Other objects will become apparent in view of the subsequent detailed description and appended claims. It has been unexpectedly found that the above objects can be accomplished by including an amino tri(lower alkylidene phosphonic acid) or water-soluble salt thereof in the boiling aqueous alkaline scouring bath in addition to the caustic material and surfactant. The amino tri(lower alkylidene phosphonic acids) have the general formula:



wherein x and y represent hydrogen or a lower alkyl containing, for example, from one to four carbon atoms. Compounds illustrative of these acids are amino tri(methylene phosphonic acid), amino tri(ethylidene phosphonic acid), and amino tri(isopropylidene phosphonic acid).

It is to be understood in addition to the acids per se, the water-soluble salts are also included within the scope of the present invention. The preferred salts are the sodium salts,

particularly the pentasodium salt. Other alkali metal salts, such as potassium, lithium and the like, as well as mixtures of the alkali metal salts may be used. In addition, any water-soluble salt, such as the ammonium salt, e.g.,



which exhibit the characteristics of the alkali metal salt may be also used to practice the invention.

It is found desirable to use at least about 0.01 percent by weight of said phosphonic acid based on the total weight of the combination of the caustic, surfactant, said phosphonic acid (or salt thereof,) and water. It is to be understood that the amount necessary depends upon the level of contamination of the scouring bath. However, the general usage of the above-mentioned amino phosphonic acids indicates a practical upper limit is about 2.0 percent by weight. The preferred range is from about 0.1 percent to about 0.5 percent.

The temperature of the bath is desirable in the range of from about 125° F. to the boiling point of the scouring solution but temperatures from about 140° F. to about 210° F. are preferred.

It is believed that the amino tri(lower alkylidene phosphonic acids) unexpectedly contribute to the scouring step by solubilizing (removing from the surface) the polymeric foreign materials on the fibers and thus speed up their emulsification, saponification, or hydrolysis by the caustic in solution which generally is sodium hydroxide. This mechanism is quite unexpected, especially since the contribution of the above-mentioned amino phosphonic acid to the removal of these foreign materials is greater than that of the surfactant. It is to be understood that the above idea or mechanism is merely a theory and is not intended to be limitative as to the scope of this invention.

The practice of the invention and the advantages provided thereby are further illustrated by the following examples which are not intended to be limitative:

One practical method to ascertain the degree of cleanliness of a textile material is to determine its whiteness. This can be accomplished by using a Gardner Automatic Color Difference Meter made by Gardner Laboratory, Inc., Bethesda, Maryland. The color difference meter directly measures color by reflectance in different scales. In this test, the color was determined relative to a standard which was as close to perfect whiteness as is possible. Utilizing this testing device, the machine is so calibrated that the control or standard material used for comparative purposes registers a *b* value to zero. When a high positive *b* value is obtained, the material is too yellow. A negative *b* value indicates blueness. In the textile industry, it is desirable to have as low a *b* value as possible, even if the material is on the blue (negative) side of the *b* scale. Too much blueness is undesirable, but it is acceptable up to a point because it means that the material has less impurities in it. These impurities, thus, cause the yellow color.

As a practical demonstration, 1 liter of boiling caustic solution containing 80.0 grams of a 50 weight percent sodium hydroxide solution and 12.0 grams of Biofax P-35, a phosphated surfactant typical of those used in the industry, were used in this experiment as the scouring bath. Six-20 gram fabric samples, two of 100 percent cotton, two of 35 percent cotton and 65 percent polyester, and two of 50 percent cotton and 50 percent polyester were tested. For each kind of fabric, one sample was scoured in the bath described above with the addition of 2.3 grams of amino tri(methylene phosphonic acid) herein referred to as ATMP, and one sample was scoured without ATMP. Each sample was scoured for one hour at 210° F. and rinsed twice with water at 210° F. for 30 minutes each time. The results are shown in the following table I.

3  
TABLE I

| Fabric                    | "b" Value    |           |
|---------------------------|--------------|-----------|
|                           | Without ATMP | With ATMP |
| 100% Cotton               | 7.5          | 6.4       |
| 35% Cotton, 65% Polyester | -0.2         | -1.2      |
| 50% Cotton, 50% Polyester | 6.8          | 4.8       |

The *b* value of the cotton fabric sample scoured with ATMP was 14.7 percent lower than the *b* value of the sample scoured without it. The *b* value of the 35 percent cotton and 65 percent polyester fabric was 600 percent lower when scoured with ATMP than when scoured without it. The *b* value of the 50 percent cotton and 50 percent polyester fabric was 29.4 percent lower with ATMP. All of the recorded *b* value differences (i.e., 1.1, 1.0, and 2.0) are significant since a 0.2 difference in *b* value is considered in the art as substantial. In fact, the color difference of 0.2 *b* value can readily be seen by visual observation.

EXAMPLE II

Another method to determine cleanliness of textiles is to determine the amount of water extractable and solvent extractable foreign matter left on the material after scouring. This is accomplished by extracting the foreign matter by rinsing the textile material with separate and individual portions of several different solvents and then finally, water. The rinse solution is then evaporated and the amount of foreign matter which was on the textile material is determined by weighing the residue. The solvents used in this experiment were trichloroethylene, ethanol and acetone, and then water.

The samples of 100 percent cotton fabric and 35 percent cotton and 65 percent polyester fabric from Example I were treated in the manner described above. Similar unscoured samples of those fabrics were also tested. The results are shown in the following table II:

TABLE II

| Fabric  | Without | With | Unscoured         |
|---------|---------|------|-------------------|
|         | ATMP    | ATMP |                   |
| % Water | 0.77    | 0.53 | 5.61 <sup>1</sup> |

4

| 5 | Extractables |             |           |              |
|---|--------------|-------------|-----------|--------------|
|   | 100% Cotton  | 35% Cotton, | 65% Poly- | Extractables |
|   | % Solvent    | 0.30        | 0.22      | 0.84         |
|   | Extractables | 0.50        | 0.43      | 6.36         |
|   | % Water      |             |           |              |
|   | Extractables |             |           |              |
|   | % Solvent    | 0.55        | 0.48      | 0.72         |
|   | Extractables |             |           |              |

10

<sup>1</sup>The higher the numerical value, the more foreign matter present on the textile material.

- 15 The scour with ATMP removed 9.5 percent more of the solvent extractables and 4.3 percent more of the water extractables from the 100 percent cotton fabric than the scour without the additive did. The ATMP scour removed 9.7 percent more of the solvent extractables and 1.2 percent more of the water extractables. These figures show a significant improvement and the differences (though numerically small) are considered significant in the art.

The above tests were carried out using amino tri(n-propylene phosphonic acid) and amino tri(n-butylene phosphonic acid) with substantially the same results.

The foregoing examples have been described in this specification for the purpose of illustration and not limitation. Many other modifications and ramifications will naturally suggest themselves to those skilled in the art based on this disclosure.

- 30 These are intended to be comprehended as within the scope of this invention.

What is claimed is:

1. In a process for treating textile materials which comprises the steps of singeing, desizing, scouring, bleaching, scouring, 35 mercerizing, dyeing or printing, and finishing, the improvement which comprises incorporating into the scouring bath, which is maintained at a temperature of from about 140° F. to about 210° F., which consists essentially of a caustic material and a surfactant, at least 0.01 percent by weight, based on the 40 total weight of the scouring bath, of a solubilizing agent which is amino tri(methylene phosphonic acid).
2. The process as set forth in claim 1 wherein the concentration of the solubilizing agent is from about 0.1 to about 0.5 percent by weight.
- 45 3. The process as set forth in claim 1 wherein the caustic material is sodium hydroxide.

\* \* \* \* \*

50

55

60

65

70

75